

1  
3,827,858

## DURABLE-PRESS COTTON TEXTILES AND METHOD OF MAKING SAME

Geoffrey A. Byrne, Haddington, Scotland, and Jett C. Arthur, Jr., Metairie, La., assignors to the United States of America as represented by the Secretary of Agriculture

No Drawing. Filed Apr. 27, 1972, Ser. No. 248,180  
Int. Cl. C08f 1/24, 3/46; D06m 13/20

U.S. Cl. 8—184

2 Claims

### ABSTRACT OF THE DISCLOSURE

Durable-press cotton textiles are prepared by a chemical process wherein methacrylic acid is grafted onto the textile and the grafted textile is subsequently crosslinked with dimethyloldihydroxyethyleneurea (DMDHEU) without the use of the usual catalysts such as zinc nitrate. The textile is dried to a moisture content of about 0.5%, irradiated in an inert atmosphere to a dosage of 0.5–1 megarad, immersed in a solution of methacrylic acid, methanol and water, washed, dried then immersed in a solution of DMDHEU, water and a wetting agent, dried and cured at 160° C.

A non-exclusive, irrevocable, royalty-free license in the invention herein described throughout the world for all purposes of the United States Government, with the power to grant sublicenses for such purposes, is hereby granted to the Government of the United States of America.

This invention relates to chemical treatments of cotton and other cellulosic textiles. More specifically, this invention relates to an improved chemical process comprising a sequence of steps useful in the preparation of durable-press fabrics wherein (1) a cotton or other cellulosic poly(vinyl) graft copolymer fabric is prepared by a free-radical initiated graft copolymerization process, and (2) the cellulosic-poly(vinyl) copolymer fabric is submitted to a crosslinking reaction without catalyst, to yield durable-press cellulosic textile products without the usual losses in breaking strength and tearing strength which generally are obtained in durable-press products.

The main object of this invention is to provide improvement in the chemical processing which yields durable press fabrics.

Another object of this invention is to provide the fabrics produced by the improvements indicated.

In the prior art cotton fabrics are commonly crosslinked with reagents such as dimethyloldihydroxyethyleneurea to obtain durable-press cotton textile products. Catalysts, such as zinc nitrate, are included in the crosslinking formulations to obtain the crosslinked textiles with good wrinkle recovery properties. The wet impregnated fabrics are cured at elevated temperatures to obtain the desired textile properties. Although the wrinkle resistance is enhanced in these treatments the breaking strengths of the finished fabrics are reduced to about one-half of the untreated fabrics, and the tearing strengths of the fabrics are reduced to about one-fifth of the untreated fabrics.

The present invention discloses a distinct improvement in the durable-press properties of cotton textiles by the preparations of cotton graft copolymers and then by crosslinking of the cotton copolymer with the usual crosslinking reagents, such as the aforementioned dimethyloldihydroxyethyleneurea, but without catalysts. We have now

2

found that the durable-press properties of the derived crosslinked cotton copolymer textile products are improved over those of crosslinked cotton textile products in that the wrinkle recovery properties are improved without large decreases in breaking and tearing strengths of the cotton textile products. Furthermore, we have now found that if catalysts are excluded in the solution containing the crosslinking reagent that the wrinkle recovery properties of the crosslinked cotton copolymer textile products are improved over those of catalyzed, crosslinked cotton textile products, while the other properties, such as breaking strengths and tearing strengths of the derived durable-press cotton textile products are about the same for both crosslinked cotton copolymer textile products and crosslinked cotton textile products.

Samples of cotton fabrics used were printcloth (about 3.1 ounces per square yard, 86 x 86 thread count) and were commercial grey cloths which had been enzymatically desized, alkali scoured, and peroxide bleached on a pilot plant scale. Samples of the cotton fabrics were dried overnight in a vacuum oven at 50° C. to a moisture content of about 0.5% and then irradiated at ambient temperature (about 25° C.) in a nitrogen atmosphere in sealed glass tubes with cobalt-60 irradiation, a convenient source of radiation, to a dosage of about one-half to one megarad to produce long-lived free radicals on the cellulose molecules which comprise the cotton. Radiation-activated cotton fabric (about 1.5 parts), now containing free radical sites on the cotton cellulose molecule, was immersed in a solution of 1.5 to 3 parts of vinyl monomer, such as methacrylic acid, 2.5 to 50 parts of water, and 47.5 to 0 parts of methanol which had been purged with nitrogen, at 25° C. for the desired reaction time from about 15 to 30 minutes to yield a cotton-poly(methacrylic acid) copolymer fabric with the desired add-on of poly(methacrylic acid) from about 7 to 49%. The cotton copolymer fabric was washed with a solution of methanol-water (equal parts) to remove unreacted vinyl monomer and then air-dried at 25° C. The add-on of poly(methacrylic acid) was determined as the increase in weight of the cotton copolymer fabric over that of an untreated cotton fabric. A typical reaction time and poly(methacrylic acid) add-on from 2.5 parts of water, 47.5 parts of methanol, and 1.5 parts methacrylic acid onto 1.5 parts of cotton fabric which had been pre-irradiated to a dosage of one megarad was: 30 minutes and 7 percent add-on. Samples of untreated cotton fabrics and of cotton copolymer fabrics were padded to a wet pick-up of 100% with a typical crosslinking solution (comprising dimethyloldihydroxyethyleneurea 18 parts, zinc nitrate catalyst 3 parts, wetting agent 0.1 part, and water 78.9 parts). For several tests the zinc nitrate catalysts were omitted from the crosslinking solution. The fabrics, padded with crosslinking solution, were dried for 3 minutes at 60° C. and then cured for 6 minutes at 160° C. The durable-press properties of the treated cotton fabrics and treated cotton copolymer fabrics were determined by standard methods of the American Society for Testing and Materials, Philadelphia Pa.

The following examples are provided to facilitate the comprehension of the invention and should not be construed as limiting the invention in any manner whatsoever.

## EXAMPLES

[Durable-press, crosslinked cotton-poly(methacrylic acid) copolymer fabrics]

| Example number                                 | Grafted polymer add-on, percent | Breaking strength, lb. | Tearing strength, g. | Wrinkle recovery angle (W+E) <sup>a</sup> , degrees |
|------------------------------------------------|---------------------------------|------------------------|----------------------|-----------------------------------------------------|
| Untreated control                              |                                 |                        |                      |                                                     |
| 1.....                                         | 0                               | 32                     | 1,000                | 180                                                 |
| Crosslinked, no catalyst <sup>b</sup>          |                                 |                        |                      |                                                     |
| 2.....                                         | 0                               | 31                     | 680                  | 190                                                 |
| Crosslinked, catalyst <sup>c</sup>             |                                 |                        |                      |                                                     |
| 3.....                                         | 0                               | 15                     | 200                  | 280                                                 |
| Grafted only                                   |                                 |                        |                      |                                                     |
| 4.....                                         | 7                               | 29                     | 570                  | 200                                                 |
| 5.....                                         | 10                              | 34                     | 610                  | 200                                                 |
| 6.....                                         | 23                              | 37                     | 420                  | 214                                                 |
| 7.....                                         | 49                              | 44                     | 400                  | 158                                                 |
| Grafted, crosslinked, no catalyst <sup>b</sup> |                                 |                        |                      |                                                     |
| 8.....                                         | 7                               | 29                     | 430                  | 243                                                 |
| 9.....                                         | 10                              | 29                     | 430                  | 236                                                 |
| 10.....                                        | 16                              | 29                     | 300                  | 235                                                 |
| 11.....                                        | 20                              | 32                     | 500                  | 232                                                 |
| 12.....                                        | 35                              | 30                     | 370                  | 236                                                 |
| Grafted, crosslinked, catalyst <sup>c</sup>    |                                 |                        |                      |                                                     |
| 13.....                                        | 22                              | 11                     | 140                  | 301                                                 |
| 14.....                                        | 25                              | 14                     | 150                  | 291                                                 |

<sup>a</sup> Determined by standard procedure, American Society for Testing and Materials, Philadelphia, Pa., ASTM Designation D1295-60T.<sup>b</sup> Crosslinked with dimethyldihydroxyethyleneurea using no catalyst. (This illustrates the process of the present invention.)<sup>c</sup> Crosslinked with dimethyldihydroxyethyleneurea using zinc nitrate catalyst.

With reference to Examples 4, 5, 6, and 7, the cotton-poly(methacrylic acid) copolymer fabrics thus prepared retained breaking strengths about equal to that of untreated cotton fabric (Example 1), showed decreases in tearing strengths, and exhibited no significant changes in wrinkle recovery angles.

With reference to Examples 8, 9, 10, 11, and 12, the crosslinked cotton-poly(methacrylic acid) copolymer fabric products thus prepared retained breaking strengths about equal to that of untreated cotton fabric (Example 1), and showed decreases in tearing strengths. These specific examples illustrate the results obtained when practicing the invention, and obviously Example 8 would be the preferred embodiment economy-wise. It must be noted that not catalyst was added in any of the 8-12 Examples. These copolymer fabric products showed increases in wrinkle recovery angles ranging up to 66 degrees over those of the untreated cotton fabric (Example 1), and 56 degrees over the crosslinked, no catalyst fabric of Example 2.

With reference to Examples 13 and 14, the crosslinked cotton-poly(methacrylic acid) copolymer fabric products thus produced, the breaking strengths and tearing strengths of the copolymer fabric products were decreased as compared with the untreated cotton fabric of Example 1, as well as the grafted only products of Examples 4-7, and the grafted, crosslinked, no-catalyst products of Examples 8-12, but were about the same as the crosslinked catalyzed fabric of Example 3. Examples 13 and 14 yielded higher wrinkle recovery angles than all the other products illustrated.

The invention can be easily comprehended by examination of the textile properties of the durable-press fabric products shown in Examples 3, 13, and 14, as compared with those of the durable-press fabric products shown in Examples 8, 9, 10, 11, and 12. The durable-press fabric product shown in Example 3 was prepared by the usual crosslinking processes. It is clearly shown that in order to obtain the desired increase in wrinkle recovery (Example 3) over that of untreated, control fabric (Example 1) or crosslinked, no catalyst fabric (Example 2), large undesirable decreases in breaking strength and tearing strength are concomitantly obtained. If a cotton copolymer fabric was prepared and then crosslinked by the usual processes (Examples 13 and 14), desirable increases

in wrinkle recovery (Examples 13 and 14) over those of untreated, control fabric (Example 1) or crosslinked, no catalyst fabric (Example 2) and even over that of fabrics crosslinked by the usual processes (Example 3) were obtained. However, as in the case of the product (Example 3), there were large and undesirable decreases in breaking and tearing strengths. The fabric copolymer products of the instant invention (Examples 8-12) which, as described above, consisted of preparing cotton-poly(methacrylic acid) copolymer and then crosslinking the cotton copolymer fabric without catalysts, exhibited desirable increases in wrinkle recovery over those of untreated, control fabric (Example 1) or crosslinked, no catalyst fabric (Example 2). It should be particularly noted that this desired increase in wrinkle recovery (Examples 8-12) by the method of the instant invention was obtained without any loss in breaking strength and much less loss in tearing strength than recorded when crosslinked fabrics prepared by the usual processes (Example 3) or even for those grafted copolymer fabrics crosslinked by the usual processes (Examples 13 and 14) were prepared to illustrate the desired increases in wrinkle recovery in a durable-press cotton product.

We claim:

1. A process for preparing a durable-press cotton fabric, which simultaneously retains high breaking strength, and particularly high tearing strength with respect to untreated cotton, the process comprising:

- (a) drying a cellulosic textile to a moisture content of about 0.5%,
- (b) irradiating the dry cellulosic textile with a radioactive source, in an inert atmosphere, to a dosage of 0.5 to 1 megarad,
- (c) immersing the irradiated cellulosic textile in a solution computed to contain proportionately, including the cellulosic textile, about 1.5 parts by weight of cellulosic textile, 1.5 to 3 parts by weight of solution of methacrylic acid, 2.5 to 50 parts by weight of water, and 47.5 to 0 parts by weight of methanol at about 25° C. for periods about from 15 to 30 minutes of time to give desired poly(methacrylic acid) add-on to the cellulosic textile, of about from 7% to 49%,
- (d) washing the unreacted material off the treated cellulosic textile with a solution of methanol and water in equal parts,
- (e) drying the reacted and washed cellulosic textile,
- (f) immersing the reacted cellulosic textile in a solution computed to consist of proportionately about 18 parts by weight of dimethyldihydroxy ethyleneurea, 0.1 part by weight of wetting agent, and 78.9 parts by weight of water and padded to about 100% wet pickup,

- (g) drying the padded cellulosic textile for 3 minutes at 60° C., and
- (h) curing the dried cellulosic textile for 6 minutes at 160° C.

2. The crosslinked cotton-poly(methacrylic acid) copolymer textile product produced by the process of Claim 1.

## References Cited

| UNITED STATES PATENTS |        |               |
|-----------------------|--------|---------------|
| 2,999,056             | 9/1961 | Tanner        |
| 3,592,686             | 7/1971 | Barber et al. |
| 3,606,993             | 9/1971 | Arthur et al. |
| 3,666,400             | 5/1972 | Lofton et al. |

WILLIAM D. MARTIN, Primary Examiner

J. H. NEWSOME, Assistant Examiner

U.S. Cl. X.R.

8-820, Dig. 18; 117-56, 76 T, 93.31, 118, 139.4, 161 UB